

Aug. 2, 1927.

1,637,619

A. LUCAS

METHOD OF PRODUCING WELDING METAL

Filed Nov. 16, 1925



INVENTOR

*Anton Lucas.*  
BY  
*Arthur C. Brown*  
ATTORNEY

Patented Aug. 2, 1927.

1,637,619

# UNITED STATES PATENT OFFICE.

ANTON LUCAS, OF KANSAS CITY, MISSOURI.

## METHOD OF PRODUCING WELDING METAL.

Application filed November 16, 1925. Serial No. 69,334.

My invention relates to a method of producing welding metal and more particularly to one involving interactions of the alumino-oxide elements of a thermic mixture within a crucible, the principal object of the invention being to effect a thorough reduction of the oxide without loss of the oxide, damage to the crucible or danger to the operator.

Generically the invention relates to the art of welding, particularly to welding railway rails, with a metal product from a mixture of iron-oxide and powdered aluminum or other reducing metal or alloy, by interaction of such elements after ignition in a crucible.

The usual method of effecting such reduction has heretofore been to place the mixture in a plugged crucible, ignite the mixture and permit the reduction to progress downwardly in the crucible. While this method has been effective in so far as the reduction is concerned, it involves objections due to the nature of the material.

Reaction of an alumino-thermic mass is violent, proceeds downward with much greater rapidity than upwardly or laterally, and when occurring in a crucible, results in the steel being quickly separated from the slag. Consequently, when reaction is initiated at the top of the crucible, steel is not available at the tap hole until the entire mass has been reduced, and while this downward reaction is rapid, this method results in a spattering of the contents, with danger to the operator and loss of material, which tends to lower the quality of the steel.

I have found that by initiating the reaction at the bottom of the crucible, these objections are overcome, a better quality of steel results, and a beneficial effect produced on the crucible which tends to prolong its life.

In connection with my improved method I employ a crucible and appurtenances, the preferred form of which is illustrated in the accompanying drawing wherein:

1 designates a crucible of the type usually employed for such purposes, preferably composed of cast iron or cast steel and having walls of sufficient thickness to carry off heat generated by the reaction carried on within it, the crucible being lined with refractory material if desired, although such lining is not an essential element with my method, for the reasons presently stated.

2 The crucible has a tap hole 2 at its lower end, preferably lined with refractory ma-

terial 3, and extending through the tap hole is the usual pin 4, having a head 5 closing the hole within the crucible. I prefer to cover the head of the pin with a bed of powdered refractory material 6 to protect it from the heat from the melting material, the structure above described being similar to that ordinarily used for such purposes.

In practicing my method, however, I place a quantity of ignition powder 7 in the bottom of the crucible, over the pin and refractory material. I then insert a tube 8 into the receptacle so that it rests on the ignition powder, and then fill the receptacle above the ignition powder and about the tube with the alumino-thermic mixture 9. I then ignite the ignition powder by dropping a match or projecting a hot rod 10 through the tube into contact with the powder. The burning powder sets up a reaction in the mixture, melting the elements. The molten steel being the heavier, settles to the bottom of the crucible, and the slag, being the lighter, floats to the top. As the reaction progresses, the slag coming in contact with the relatively cold wall of the crucible, is chilled and adheres to the crucible, forming a coat thereover, which protects the crucible from the molten steel and confines the heat.

It is apparent that as the reaction starts from the bottom and progresses upwardly through the mass in the crucible, the spattering is avoided. The reaction is slower but less violent and separation of the elements more thorough and the natural separation of the elements of different gravity results in the slag lining the crucible in advance of level of the molten steel, thereby affording better protection for the crucible than in a method wherein the reaction is initiated in the top of the mass and progressed downwardly.

What I claim and desire to secure by Letters-Patent is:

1. The method of effecting alumino-thermic reaction, consisting of locating an ignition element in the bottom of a crucible, locating an ignition conduit above said element, locating an alumino-thermic mixture within the crucible above the ignition element and about the conduit, and passing an igniting element through the conduit to the ignition element.

2. The method of effecting alumino-thermic reaction, consisting of locating an

alumino-thermic mixture in a crucible, locating an ignition element below the surface of the said mixture, locating an ignition conduit above the ignition element, and passing an igniting element through the conduit to the ignition element.

3. The method of effecting alumino-thermic reaction, consisting of locating an

alumino-thermic mixture in a crucible, locating an ignition element below the surface <sup>10</sup> of said mixture, locating an ignition conduit in communication with said ignition element and passing an igniting element through the conduit to the ignition element.

In testimony whereof I affix my signature.

ANTON LUCAS.